

Jan. 12, 1965

W. H. OWEN ET AL

3,165,267

COMMINUTION AND BENEFICIATION OF REFRACTORY FLOUR

Filed June 29, 1962



FIG. 1

INVENTORS  
WILLIAM H. OWEN  
ROBERT K. SCOTT  
BY *William H. Owen*  
ATTORNEY

1

3,165,267  
COMMINUTION AND BENEFICIATION OF  
REFRACTORY FLOURWilliam H. Owen and Robert K. Scott, Pittsburgh, Pa.,  
assignors to Harbison-Walker Refractories Company,  
Pittsburgh, Pa., a corporation of Pennsylvania

Filed June 29, 1962, Ser. No. 206,373

8 Claims. (Cl. 241—24)

This invention relates to comminution and beneficiation of refractory flour, and more particularly, to a method of producing very high purity refractory flour having utility as an investment molding material.

In precision casting of metal parts by the so-called "lost wax" process, it is conventional to use a very finely divided refractory flour and a binder solution to make a pre-coat slurry. For example, an expendable, fusible, wax-like pattern is made, the dimensions of which are substantially identical in all respects to a metal part which is to be cast. This pattern is sequentially dipped into the pre-coat slurry of refractory flour and binder, the excess slurry drained therefrom, and while still wet, subjected to a stuccoing or sanding with a coarse refractory grit. This sequence of steps is repeated the number of times necessary to fabricate a shell or sheath of a desired thickness about the expendable pattern. The expendable pattern is then melted out, leaving the desired mold.

This ceramic mold is usually of very thin wall section, i.e.  $\frac{3}{16}$  to  $\frac{1}{4}$ ", is usually mounted in some manner of back-up such as sand or steel shot either loosely consolidated or unconsolidated, and has molten metal poured therein to produce the precision casting desired. These molds are used for but one casting.

The surface finish and quality of precision castings made from these molds is affected if, in any of the pre-coat slurries used, there exists occluded gases from such as air entrapped by poor mixing techniques, from gases generated by reactions between the refractory materials and the binder solution, etc.

The incidence of reaction between the refractory materials and binder solutions is considerably increased when the mold is rapidly heated to a high temperature during its contact with molten metal being cast. It is not uncommon for this molten metal to be poured into the mold at a temperature of 2900° F. and even higher. The gases which are generated under such high temperature conditions cause pinholing of the metal casting. Furthermore, they sometimes cause reaction between the molten metal and the material of which the mold is made, in such a manner as to cause spaced areas of adhesion between the casting and the mold upon cooling. Such adhesion, during cooling, causes fissures or cracks to occur in the cast shape, because of variances in the surface tension of the cooling metal. Irony materials are one of the primary causes of such gaseous exudate and surface adhesion. Even in extremely small amounts, i.e. fractions of 1%, the irony materials are detrimental.

Accordingly, it is an object of this invention to provide an improved method of comminution and beneficiation of refractory flour having particular utility as an investment molding media. It is another object of this invention to provide investment molding media substantially entirely free of those impurities which would tend to react with binder solutions or which would, under conditions of high temperature, produce gas which would pinhole or otherwise damage a precision casting.

It is yet another object of this invention to provide a very finely divided, refractory flour having less than about 0.001% metallic iron, on the basis of an oxide analysis. And it is still another object of this invention to provide very finely divided, iron-free mullite flour having par-

2

ticular utility as an investment molding media for the so-called "lost wax" and like processes.

Briefly, according to one embodiment of this invention, a technical grade mullite (calcined bauxite substantially entirely of mullite phase with minor amounts of corundum and glass) is provided, which has essentially less than 0.001%, by weight, metallic iron on the basis of an oxide analysis. This material is prepared by a process, which includes an initial crushing of a calcined feed to a mixture which is substantially all —16 mesh Tyler. This crushed material is subjected to an initial screening step, which provides three fractions. The first fraction is oversize or +16 mesh Tyler, which material is returned to the initial crushing step. An intermediate fraction is —16+48 mesh Tyler, and is subjected to subsequent treatment steps. The —48 mesh Tyler fraction is discarded.

The intermediate —16+48 mesh fraction is subjected to magnetic separation, and thence to further comminution in a ceramic-lined ball mill. The product of the ceramic mill is substantially all —150 mesh Tyler, and is termed a "flour" in the art, which flour is substantially entirely free of irony materials.

A better understanding, other features, and further objects and advantages of this invention will become obvious, to those skilled in the art, from a study of the following detailed description with reference to the drawings. In these drawings:

FIG. 1 is a schematic diagram of a preferred method of producing very finely divided beneficiated refractory flour, according to the concepts of this invention;

FIG. 2 is a schematic diagram of an alternative method. The present invention is applicable to almost all refractory materials which are capable of being reduced to a flour for use in such as investment molding procedures. It is, thus, applicable to silica, alumina-silica, alumina, zircon, zirconia, calcia, periclase, periclase-silica, chrome, chrome-periclase, etc., and like minerals. For the purposes of explanation, however, this invention will be described in the manufacture of a very finely divided, beneficiated mullite flour from calcined bauxite (an alumina-silica type mineral).

As noted above, one of the primary purposes of the invention is to remove certain gas-forming agents, such as metallic iron and irony compounds, which would react in service to produce undesired effects on a metal part being cast. In actual laboratory tests on refractory investment materials, it was found that metallic iron, in amounts of only 50 parts per million, was objectionable since it caused a sufficient volume of gas to be given off in service as to damage a precision casting.

Further, metallic iron reacts with water and other combined hydrogen present in investment molding binder solutions, to produce hydrated iron oxide and hydrogen gas. This iron oxide, when first formed, is almost colloidal in nature, and is capable of diffusing through an investment mold, to appear on the working surface thereof as a scum or stain. This stain is capable of reacting with ferrous metals being cast, according to the following general equations:



These reaction products often promote adherence of the investment molds to ferrous castings causing fissures to appear in the castings upon cooling.

The hydrogen gas, mentioned above, is a reaction product of metallic iron and water or other combined hydrogen, and coalesces to form small bubbles within the investment mold. These coalesced bubbles appear

as small gas cavities within the mold which rupture upon heating to cause fissures through the working face of the mold into which molten metal will flow, resulting in a pimpled surface on the resulting casting.

Although some of the metallic iron and irony materials found in the refractories used for investment molding are naturally-occurring, most of it appears to be picked up during grinding thereof to obtain the desired very finely divided flour state. Most of this contamination appears in the extremely fine fractions of this flour, and in such a range as to be incapable of separation by magnetic treatment.

Referring now to FIG. 1, according to this invention a quantity of bauxite having the following typical analysis (all parts by weight, and on the basis of an oxide analysis):

|                                                                               | Percent |
|-------------------------------------------------------------------------------|---------|
| Silica ( $\text{SiO}_2$ )                                                     | 15.5    |
| Alumina ( $\text{Al}_2\text{O}_3$ )                                           | 54.6    |
| Titania ( $\text{TiO}_2$ )                                                    | 1.9     |
| Iron oxide ( $\text{Fe}_2\text{O}_3$ )                                        | 0.8     |
| Calcium oxide ( $\text{CaO}$ )                                                | 0.1     |
| Magnesia ( $\text{MgO}$ )                                                     | Trace   |
| Alkalies ( $\text{Na}_2\text{O} + \text{K}_2\text{O} + \text{Li}_2\text{O}$ ) | 0.1     |
| Loss on ignition                                                              | 27.2    |

was calcined to remove all free and substantially all chemically combined water, and to produce a calcined material having an ignition loss on the order of up to about 0.1%. This calcining step may be carried out in such as a rotary kiln. The calcined material is fed to an initial crushing step in a dry pan to produce a material substantially all of which is -16 mesh Tyler. Of course, if desired, a ball mill, rod mill, impact crushing mill, etc., can be used for this step. From the dry pan, the material passes to a screening step. The screening step may be conducted in such as the Rotex screen of the Orville-Simpson Company, which is described on page 958 of the Chemical Engineers Handbook, 3rd Edition.

Three fractions result from the screening step. The first is a +16 mesh Tyler or oversize fraction, which is recycled to the dry pan. The third fraction is a -48 mesh Tyler or undersize fraction, which is disposed of.

The intermediate or -16+48 mesh Tyler fraction is passed to a magnetic treatment to remove all of the iron and irony fluxes contained therein. In this treatment, the material is sequentially subjected to a permanent magnet pulley or drum-type separator, an electromagnetic pulley-type separator, and then to a second permanent magnet-type separator.

The sequence of permanent magnetic and electromagnetic treatment steps produces a product having essentially less than 0.001%, by weight, metallic iron and irony materials. This material is fed to a ceramic lined mill of the ceramic ball mill type to produce a refractory flour. The product from the ceramic ball mill is fed to suitable storage facilities, such as a storage hopper, for subsequent packaging as desired.

Previously, it has not been thought commercially feasible to produce investment molding flour by ceramic milling, because of the great expense involved in large ceramic mill installations. However, by our preliminary separation and isolation of an intermediate pre-ground fraction, particularly amenable to magnetic separation treatment, all of the material which is passed through the ceramic mill is product and there is no crushing of material which must be subsequently wasted.

An alternative flow sheet, schematically shown in FIG. 2, is useful for treating smaller quantities of material. It includes an initial calcining step, a crushing step to produce a substantially -28 mesh Tyler material, a first screening step to remove the oversize or +28 mesh fraction for recycle to the crusher, a subsequent 100 mesh screening step to remove a -100 mesh waste prod-

uct, with an intermediate -28+100 mesh fraction being subjected to a magnetic separation treatment (which may be similar in all respects to the magnetic separation treatment shown in FIG. 1). The -28+100 mesh fraction is subsequently passed to a ceramic mill to produce an iron-free ceramic flour.

The method schematically indicated in FIG. 1 is preferable for an industrial scale operation, since the extremely fine -100 mesh waste of the method of FIG. 2 is more difficult to handle than the -48 mesh fraction of the method of FIG. 1. In any event, the fraction which passes to the magnetic separating step must be entirely +100 mesh, and is preferably all less than 16 mesh.

Two samples of mullite flour, which were actually produced according to the method of FIG. 1, were subjected to a very careful chemical analysis in a laboratory. The first sample was substantially entirely -150 mesh Tyler and the second was substantially entirely -200 mesh Tyler. Each of the samples was divided into two parts. A first part of each sample was tested qualitatively for the presence of iron or irony substances, by wetting with water and adding concentrated hydrochloric acid. There was no evidence of gas evolution from either of the samples, as would have indicated the presence of iron.

Quantitative chemical tests were then undertaken on the second portion of each of the samples. The -150 mesh sample indicated 0.0002%, by weight, iron present. No evidence of iron could be found in the -200 mesh sample.

The following is a brief synopsis of the method used to quantitatively analyze the material for metallic iron:

A 100.0 gram sample of material, as received, was transferred to a 250 ml. Erlenmeyer flask, and 50 ml. of 4%  $\text{HgCl}_2$  solution was added. Using a trap to collect the condensate and a burner to ignite the exit gas, the air was displaced from the flask by a continuous flow of natural gas. Both the flask and sample were heated for 10 minutes, to just below boiling of the sample. The flask was then cooled in ice water and the solution decanted through a 5 cm. #2 Whatman paper in a #1 Büchner funnel into a 250 ml. flask containing 15 ml. of 1-1  $\text{H}_2\text{SO}_4$ . The sample was washed by decantation using 25-30 ml. of cold water for each decantation. The filtrate was transferred (225 ml.) to a 600 ml. beaker and titrated with a standard  $\text{Ce}(\text{SO}_4)_2$  solution using one drop of o-phenanthroline as an indicator. It was then titrated to a colorless end-point. The sample was washed and the filtrate added to the titrated solution until the indicator showed no color change, or 1 drop of  $\text{Ce}(\text{SO}_4)_2$  was sufficient to discharge the color, to assure complete removal of ferrous salts from the sample. 0.1 ml. from the titration was deducted for the blank, and percentage of iron was calculated.

Calculation:

$$\frac{\text{ml.} \times 0.2239}{\text{wt. sample}}$$

Note.—Preparation of  $\text{Ce}(\text{SO}_4)_2$  solution (0.05 N):

8.4 grams of  $\text{Ce}(\text{SO}_4)_2$  were dissolved in a solution containing 14 ml. of  $\text{H}_2\text{SO}_4$  and 300 ml. water. It was then filtered through a #5 Whatman paper using suction, diluted to 500 ml. and mixed well. Treated as described above, it was standardized against 0.0100 to 0.0200 gram of iron wire.

In an actual industrial test using iron-free mullite flour, produced according to the method of FIG. 1, very high quality precision castings were obtained. In addition to the precision of the castings obtained in the absence of metallic iron and irony substances, it was discovered that a mold made of such a material resisted wetting by the molten metal. It is surmised that wetting, which had been noted with previous molding materials,

had been the result of deposits of iron material on the working surface of the mold, which encouraged wetting of the mold by the molten metal. However, with the iron-free material of this invention, wetting was not noted.

Having thus described the invention in detail and with sufficient particularity as to enable those skilled in the art to practice it, what we desire to have protected by Letters Patent is set forth in the following claims.

We claim:

1. Method of producing a refractory flour essentially free of iron material for use as an investment molding media, which comprises the steps of passing a selected refractory material to a preliminary size reduction stage, isolating an intermediate fraction substantially all of which rests on a 100 mesh Tyler screen from the reduced material, removing substantially all iron material from the intermediate fraction, passing the resulting material to a secondary size reduction treatment in a ceramic mill, said secondary size reduction treatment producing a refractory flour substantially all of which is -150 mesh Tyler and substantially entirely free of iron materials.

2. Method of claim 1, in which the selected refractory material is bauxite.

3. Method of producing a refractory flour essentially free of iron material for use as an investment molding media, which comprises the steps of passing a selected refractory oxide material to a calcining stage, passing the calcined material to a preliminary size reduction stage, isolating an intermediate fraction substantially all of which rests on a 100 mesh Tyler screen from the reduced material, removing substantially all iron material from the intermediate fraction, passing the resulting material to a secondary size reduction treatment producing a refractory flour substantially all of which is -150 mesh Tyler and substantially entirely free of iron materials.

4. Method of claim 3, in which the refractory material is bauxite.

5. Method of producing a refractory flour essentially free of iron material and having particular utility as an investment molding media, which comprises the steps of passing a selected refractory oxide to an initial crushing step to produce a material which is substantially all -16 mesh Tyler, passing the crushed material to a separation stage, said separation stage dividing the crushed material into three fractions, the first fraction being +16 mesh Tyler oversize, returning said oversize to the crushing step, a second fraction being -100 mesh Tyler and undersize, the third fraction being an intermediate -16+100 mesh Tyler fraction, passing the intermediate fraction to a magnetic separation treatment, in which substantially all iron material is removed, passing the iron-free intermediate fraction to a fine crushing stage in a ceramic mill to thereby produce a refractory flour substantially free of iron materials.

6. Method of producing a refractory flour essentially free of iron material and having particular utility as an investment molding media, which comprises the steps of

calcining a selected refractory oxide material to remove all free water and substantially all chemically combined water, passing the calcined material to a separation stage, said separation stage dividing the crushed material into three fractions, the first fraction being +16 mesh Tyler oversize, returning said oversize to the crushing step, a second fraction being -100 mesh Tyler and undersize, the third fraction being an intermediate -16+100 mesh Tyler fraction, passing the intermediate fraction to a magnetic separation treatment, in which substantially all iron material is removed, passing the iron-free intermediate fraction to a fine crushing stage in a ceramic mill to thereby produce a refractory flour substantially free of iron materials.

5 7. Method of producing a refractory flour essentially free of iron material for use as investment molding media, which comprises the steps of passing a selected refractory material to a preliminary size reduction stage, isolating an intermediate fraction substantially all of

10 which passes a 16 mesh screen and rests on a 100 mesh screen, treating said material to reduce the iron content thereof to essentially less than 0.001%, passing the resulting material to a secondary size reduction treatment in a ceramic mill, said secondary size reduction treatment

15 producing a refractory flour all of which is -150 mesh Tyler and substantially entirely free of iron materials.

20 8. Method of producing a refractory flour essentially free of iron material and having particular utility as an investment molding media, which comprises the steps of

25 passing a selected refractory oxide to an initial crushing step to produce a material which is substantially all -16 mesh Tyler, passing this crushed material to a separation stage, the separation stage dividing the crushed material into three fractions, the first fraction being substantially

30 +16 mesh Tyler oversize, returning said oversize to the crushing step, a second fraction being -100 mesh Tyler and undersize, discarding said undersize, the third fraction being an intermediate -16+100 mesh Tyler fraction, passing this intermediate fraction to a magnetic

35 separation treatment in which the iron material content is reduced to less than 0.001%, passing this iron-free intermediate fraction to a fine crushing stage in a ceramic mill to thereby produce a refractory flour substantially free of iron materials.

40

35 9. Method of producing a refractory flour essentially free of iron material and having particular utility as an investment molding media, which comprises the steps of

45 10. Method of producing a refractory flour essentially free of iron material and having particular utility as an investment molding media, which comprises the steps of

50 11. Method of producing a refractory flour essentially free of iron material and having particular utility as an investment molding media, which comprises the steps of

55

#### References Cited by the Examiner

##### UNITED STATES PATENTS

|           |       |              |       |           |
|-----------|-------|--------------|-------|-----------|
| 1,898,371 | 2/33  | Hutchins     | ----- | 241-24 X  |
| 2,269,912 | 1/42  | Ladoo et al. | ----- | 241-24    |
| 2,468,321 | 4/49  | Bland        | ----- | 241-24    |
| 2,603,423 | 7/52  | Buehl        | ----- | 241-24 X  |
| 2,618,530 | 11/52 | Gardner      | ----- | 106-38.27 |
| 2,840,480 | 6/58  | Stoddard     | ----- | 106-38.27 |
| 2,865,570 | 12/58 | Nutting      | ----- | 241-24    |

J. SPENCER OVERHOLSER, Primary Examiner.

MORRIS LIEBMAN, Examiner.